

# UNITED STATES PATENT OFFICE.

JOSEPH M. FLANNERY, OF PITTSBURGH, PENNSYLVANIA, ASSIGNOR TO STANDARD CHEMICAL COMPANY, OF PITTSBURGH, PENNSYLVANIA.

## HIGH-SPEED STEEL.

1,210,626.

Specification of Letters Patent.

Patented Jan. 2, 1917.

No Drawing.

Application filed February 19, 1916. Serial No. 79,431.

To all whom it may concern:

Be it known that I, JOSEPH M. FLANNERY, a citizen of the United States, and a resident of Pittsburgh, in the county of Allegheny and State of Pennsylvania, have invented certain new and useful Improvements in High-Speed Steel; and I do hereby declare the following to be a full, clear, and exact description of the invention, such as will enable others skilled in the art to which it appertains to make and use the same.

This invention relates to improvements in steel alloys, and more particularly to high speed steel,—one object of the invention being to produce a high speed steel which shall have added to the qualities of tungsten thereof, similar qualities derived from the addition of another alloying metal which shall serve to materially reduce the quantity of tungsten used and at the same time increase the quality of the product in strength, ductility and heat-resisting properties, and enhance its efficiency for use as high speed tool steel.

With this and other objects in view, the invention consists in a certain novel high speed steel alloy as hereinafter set forth and pointed out in the claims.

The invention further consists in tungsten steel having uranium alloyed therewith.

In the manufacture of my improved high speed steel, I alloy with tungsten steel, uranium in a proportion appreciably less than that of tungsten. It is now common practice in the manufacture of tungsten steel, to incorporate into a body of steel a quantity of tungsten approximately equal to from 12 to 18 per cent. of the finished product. This large proportion of tungsten renders the cost of manufacture of tungsten steel very expensive, and it is the aim of my invention to reduce the cost of such steel by reducing the proportion of tungsten necessary in its manufacture and at the same time increase the efficiency of the product in all qualities incident to high speed steel.

I have found that by incorporating an amount of uranium not exceeding three per cent. into tungsten steel containing as low as eight per cent. tungsten, a high speed steel is produced having all the qualities of tungsten steel containing eighteen per cent.

tungsten, and that the uranium gives to the product greater efficiency, toughness, thermal absorption, and less brittleness. An even smaller proportion of uranium than three per cent. may be used with good results.

In the manufacture of my improved high speed steel, I may employ either ferro-uranium or uranium metal, which should be added to the bath of molten steel from five to ten minutes before pouring, after de-sludging and after all other alloys have been added. The steel should be poured as soon as the uranium has become melted,—this usually requiring from five to ten minutes unless an electric furnace be employed rather than a crucible when less time will be required for the melting of the uranium.

The presence of uranium in tungsten steel, not only greatly reduces the proportion of tungsten necessary, thus reducing the cost of tungsten content and cost of manufacture of the high speed steel, but it also enhances the hardness, toughness, thermal absorption and general efficiency and durability of the product for the manufacture of cutting tools. The alloy may be crushed to the desired size and applied to the molten mass while pouring in the ladle, or after the molten mass is in the ladle. It may also be applied in the crucible or furnace.

Having fully described my invention what I claim as new and desire to secure by Letters-Patent, is:—

1. High speed tungsten steel having uranium alloyed therewith, the uranium replacing a portion of the tungsten used in ordinary tungsten steel.

2. High speed steel containing tungsten and uranium in approximately the relative proportions specified.

3. High speed tungsten steel having uranium alloyed therewith in proportion less than the proportion of the tungsten content, the uranium replacing a portion of the tungsten used in ordinary tungsten steel.

4. High speed tungsten steel, having uranium alloyed in a proportion as high as three per cent. uranium, the uranium replacing a portion of the tungsten used in ordinary tungsten steel.

5. High speed tungsten steel, containing

approximately eight per cent. tungsten and approximately three per cent. uranium.

6. High speed steel, containing tungsten and uranium, the proportion of uranium being less than one-third the proportion of tungsten.

In testimony whereof, I have signed this

specification in the presence of two subscribing witnesses,

JOSEPH M. FLANNERY.

Witnesses:

WILLIAM GANLEY,  
H. B. KEARNEY.